

July 23, 1929.

J. R. WILSON

1,722,121

ELECTRON DISCHARGE DEVICE

Filed June 25, 1925



Inventor:  
James R. Wilson  
by *Edward A. Atty.*

Patented July 23, 1929.

## UNITED STATES PATENT OFFICE.

JAMES R. WILSON, OF NEW YORK, N. Y., ASSIGNOR TO WESTERN ELECTRIC COMPANY,  
INCORPORATED, OF NEW YORK, N. Y., A CORPORATION OF NEW YORK.

## ELECTRON-DISCHARGE DEVICE.

Application filed June 25, 1925. Serial No. 39,447.

- This invention relates to electron discharge devices and has for an object the prevention of secondary electron emission from the grid of a vacuum tube.
- 5 In devices of this character provided with a thermionically active coated filament, the high operating temperature of the filament causes particles of the active coating to vaporize, some of which deposit on the grid.
- 10 This deposit prevents the proper operation of the tube, since the heat of the grid causes the deposit thereon to emit electrons. This grid emission causes a "blocking effect" on the electron stream, thereby paralyzing the
- 15 continued operation of the device.
- This blocking is eliminated in accordance with this invention, by providing on the grid, a coating which combines with the thermionically active particles thrown off the filament to form compounds or compositions which are not thermionically active at the temperature of the grid. In a tube having an alkaline earth oxide coated filament, a coating preferably of aluminum is formed
- 20 on the grid which completely prevents emission from the grid as it combines with the alkaline earth metals or oxides to form aluminates which are thermionically inactive compounds. A further function of this
- 25 coating is to aid in cleaning up the tube during operation by fixing the oxygen or other gases within the tube.
- Referring to the drawing the single figure illustrates an electron discharge device equipped with a control electrode treated in accordance with this invention.
- The electron discharge device as illustrated, comprises an evacuated glass vessel 10, to which the usual base portion 11 is attached. This base portion provides a support for suitable terminals 12. Within the vessel 10 is a glass stem 13 from which an arbor 14 arises. This arbor provides means for supporting an anode 15, a grid 16, and
- 40 a filament 17 having an alkaline earth oxide coating, preferably formed of barium and strontium oxides. The anode, as shown, is in the form of a flattened cylinder and is supported by suitable wires (not shown) extending from the arbor 14. A wire grid 16
- 45 is positioned within the anode 15 and is supported from the arbor by wires 18. The cathode or filament 17 is placed within the grid and supported from the upper end of
- 50 the arbor by the resilient wire hooks 19.
- This filament is supported at the lower end by resilient connections 20, 21, and 22, the wires 20 and 22 also acting as the leading-in wires. The wires 23 and 24 are connected respectively to the grid and anode. These 60 wires are sealed to the glass stem 13 and are connected to the terminals 12 in any well-known manner.
- In the manufacture and preparation of the electrodes for assembly within the evacuated vessel, the control electrode or grid 16 may be made of any desirable material such as nickel, iron or chromel. The grid, in accordance with this invention, is given a treatment whereby an aluminum coating is 70 formed thereon, which, in the operation of the device, combines with particles thrown off the filament to form a compound or composition which is not thermionically active. As it is somewhat difficult to apply aluminum alone to the grid, it is coated with a mixture of powdered aluminum and pulverized fused aluminum oxide, the latter product being commercially known as "alum-dum," and acting somewhat in the nature of 75 a binding. This method of coating is known as calorizing in the metallurgical art. One method of coating the grid in accordance with this invention, is to provide a powdered mixture of approximately 50% aluminum and 50% of pulverized fused aluminum oxide. This mixture is placed in a nickel 80 box and one or a number of grids are embedded in the powdered mixture. The grids are preferably preglowed before inserting in 85 the powdered mixture to remove surface oxides and occluded gases. After embedding the grids in the powdered mixture the box may be placed in an electric oven and a stream of hydrogen passed over the box for 90 a period of twenty minutes. The heating current is turned on and the material held at a temperature of approximately 850° C. for about one and a half hours. This treatment provides a thorough coating of the 100 metal grid and forms a bright hard coating which has a flaky appearance. This coating is substantially non-porous in structure yet highly absorbent as to its gas fixing characteristics.
- 105 The calorized grid, when assembled in an electron discharge device performs the ordinary function of a control electrode notwithstanding the hard insulating coating on the grid, while the oxide coating forms an 110

insulating wall between the grid and the filament whereby any particles thrown off from the filament will be taken up by the aluminum or aluminum oxide coating to 5 form a compound of barium or strontium aluminate or a composition of these aluminates which is not an emitter of electrons. This arrangement considerably improves the 10 operation of electron discharge devices, since the taking up of active particles by the grid tends to annul the further operation of the control electrode, because that electrode becomes an electron emitter, thereby blocking the electron stream to the anode. 15 Due to the presence of the aluminum, either alloyed with the grid or suspended in the oxide coating, a continuous cleaning up effect is carried on during the operation of the device, since the gases evolved from the 20 electrodes are absorbed by the aluminum which has "getter" properties. This function of the coating considerably increases the life and activity of the filament by fixing the occluded gases and maintaining a high 25 degree of evacuation in the device.

Although a particular mixture of the composition has been disclosed, it is apparent that the coating may be modified to suit various conditions so long as the final coating contains free aluminum. Furthermore,

it is also within the scope of the invention to alloy aluminum with the metal of which the grid is composed.

What is claimed is:

1. An electron discharge device comprising 35 a cathode having a thermionically active coating, a grid and an anode, said grid being coated with a material capable of combining with particles from said cathode to form a thermionically inactive compound 40 and capable of fixing gases evolved within the device.

2. An electron discharge device comprising 45 an alkaline earth oxide coated cathode, a grid and an anode, and a coating on said grid, said coating containing aluminum.

3. An electron discharge device comprising 50 an oxide coated cathode, a grid and an anode, said grid having a coating containing aluminum and aluminum oxide.

4. An electron discharge device comprising 55 an alkaline earth oxide coated cathode, a grid, and an anode, said grid having a coating capable of combining with said alkaline earth oxides thrown on the grid to form aluminates which are thermionically inactive compounds.

In witness where, I hereunto subscribe my name this 23d day of June, A. D. 1925.

JAMES R. WILSON.